

# UNITED STATES PATENT OFFICE.

EUGENE DU PONT, OF WILMINGTON, DELAWARE, ASSIGNEE TO E. J. DU PONT DE NEMOURS & CO., OF SAME PLACE.

## EXPLOSIVE COMPOUND.

SPECIFICATION forming part of Letters Patent No. 363,827, dated May 31, 1887

Application filed June 5, 1885. Serial No. 167,747. (No specimens.)

To all whom it may concern:

Be it known that I, EUGENE DU PONT, a citizen of the United States, residing at Wilmington, in the county of New Castle and State of Delaware, have invented a new and useful Compound, principally for use in guns of medium and large caliber, of which the following is a specification.

The first object of my invention is to obtain an explosive which shall have great ballistic force, and its second object is to obtain a powder which shall obviate, as far as possible, the many disadvantages pertaining in a greater or less degree to all artillery explosives, and which consists in the smoke arising from the burning powder, such smoke obscuring the view and interfering with the sighting for a second shot.

I have found by experiment that substances having in their component parts the elements of hydrogen and oxygen in such proportions that, upon being released from the rest of the component parts by combustion, they will combine to form water and steam, and greatly increase the explosive force of the powder of which they form a constituent element. The action of such powders seems to be as follows: Upon firing the charge the gases confined in the powder are released and act to expel by their expansion the projectile toward the muzzle of the gun. This I term the "first explosion." At this time the oxygen and hydrogen are released as gases, but under too great heat to unite in the form of steam. As the pressure is decreased by the motion of the projectile in the gun, this heat also decreases, and the gases (oxygen and hydrogen) unite in the form of water. The heat generated by this union at once changes the water into steam, and this expansion, which takes place before the projectile leaves the muzzle of the gun, I term the "second explosion." There is thus formed a powder of great explosive force which acts twice upon the projectile. I have also found that such powders are very effective in dissipating the smoke arising from the discharge, owing, as I suppose, to the fact that the steam, generated as above stated, condenses, and in so doing absorbs large quantities of the carbonate of potash, the solid portion of the result of decomposition of a charge

of powder and that portion which forms the smoke.

Thus I employ in place of the carbon usually used in the composition of explosive powders the substances known as "carbohydrates," and which have the chemical formula of cellulose,  $(C_6H_{10}O_5)_n$ , or an approach to it--such as wood pulp, starch, dextrine, &c., or other substances, such as sugar, having substantially the chemical formula of  $C_{12}H_{22}O_{11}$ . All such substances having substantially the formulas aforesaid, and the capacity of forming water and steam by the action of the explosion, I term in this specification "carbohydrates." Instead of using one substance having the required chemical formula, two or more may be used having the necessary elements separate, which, when liberated, will combine to form steam and act in the manner required.

The materials should be mixed in a finely-divided condition, and it is better to mix the carbohydrates with the other ingredients of the powder after such other ingredients have been mixed, as such carbohydrates are apt to be gummy in their nature.

I have found, for example, that a very effective powder may be made of the following substances, in substantially the proportions specified, viz: Saltpeter, (for which other known nitrates may be substituted,) seventy-eight parts; sulphur, 2.8 to 3 parts; carbohydrates, three to four parts; charcoal retaining its fibrous structure, 12 or 12.5 parts. This powder, to be most effective, should be made in prismatic grains, and I have found that the best results are obtained by so constructing said grains that they are less dense in the middle than at the ends, which therefore have the particles more compacted together at those points than in the middle. My method of making these grains of such varying density is described in an application for Letters Patent filed August 12, 1885, Serial No. 167,749. Such form and construction of the grains retards the development of the gases from combustion until it is desired to obtain the maximum force, and I find that the fibers of the charcoal retaining its fibrous structure referred to materially aid in this result, as they tend to

prevent the grains of powder from becoming broken up. The use of charcoal retaining its fibrous structure, as above referred to, forms the subject of an application for Letters Patent filed June 5, 1885, Serial No. 167,748.

What I claim is—

1. An explosive compound consisting of a nitrate, sulphur, charcoal retaining its fibrous structure, and a carbohydrate, substantially as described.

2. An explosive compound consisting of saltpeter, sulphur, charcoal retaining its fibrous structure, and sugar, substantially in the proportions specified.

EUGENE DU PONT.

Witnesses:

J. E. HINDON HYDE,  
THOMAS HUNT.